

# UNITED STATES PATENT OFFICE.

FERDINAND E. CANDA, OF NEW YORK, N. Y.

## JOURNAL AND OTHER BEARINGS.

SPECIFICATION forming part of Letters Patent No. 269,636, dated December 26, 1882.

Application filed August 11, 1882. (No specimens.)

*To all whom it may concern:*

Be it known that I, FERDINAND E. CANDA, of the city, county, and State of New York, have invented a new and useful Improvement 5 in Journal and other Bearings, of which the following is a full, clear, and exact description.

This invention has for its object the production of an improved anti-friction bearing for journals and other moving parts of machinery— 10 that is, a bearing by which the friction and wear of the moving parts in contact will be greatly reduced.

The invention consists in a bearing composed of a metallic compound or alloy in the 15 form of an amalgam, with or without other substances held in mechanical combination, substantially as herein described.

To carry my invention into practical effect I take any of the well-known metals or alloys 20 used for forming bearings, and which will amalgamate with mercury—such as bronze or copper, tin, lead, and antimony—either separately or in the form of a metallic compound, and reduce the said metals or alloys to a powder 25 in any suitable crushing and pulverizing mill. If the metals are separately pulverized, they are then mixed together in any desired proportions. I then add to the pulverized metallic masses or mixtures about an equal 30 amount of mercury—that is to say, to one hundred parts in weight to the pulverized metallic mass or mixture I add about one hundred parts of mercury. This is done in any suitable vessel or mixer and the mercury 35 thoroughly stirred up with the pulverized metals to bring the whole mass to an amalgam, artificial heat, say of 280° Fahrenheit, being used, if desired, to hasten the operation. Said amalgam, while in a plastic state, is then removed 40 to a mold or molds of the required shape of the bearing to be produced, and pressure applied to give it form and to expel all superfluous

mercury, after which the amalgam-bearing is allowed to harden, when it is ready for use. A bearing thus produced will be found to have 45 very superior anti-friction properties, the mercury contained in it being a most important factor—in fact, a prime one. It may, however, be still further improved, if desired, by adding to the pulverized metals or metallic mixtures, 50 during the hereinbefore-described process of making the bearing, a certain amount of pulverized graphite—say from five to ten parts in weight—to either of the pulverized metallic mixtures hereinbefore named, and well mixing 55 the same with the pulverized metals before the amalgamation takes place, and subsequently subjecting the whole mass to pressure and allowing it to harden, as before described. Such graphite, although only mechanically combined 60 with the amalgam, will, by its well-known properties, give a self lubricating- or greasy, soft, and smooth character to the bearings. Other lubricating substances—such as mica or soapstone—might be mechanically combined 65 with the amalgam in like manner.

By tempering the pressure applied to the amalgamated mass while in the molds the amount of mercury retained in the mass may be regulated as required. 70

Having thus described my invention, I claim as new and desire to secure by Letters Patent—

1. A journal or other bearing composed of mercury and other suitable metals amalgamated therewith, substantially as specified. 75
2. A journal or other bearing composed of mercury and other suitable metals amalgamated therewith, and a lubricating substance mechanically combined with the amalgam, essentially as set forth.

FERDINAND EUGENE CANDA.

Witnesses:

JAMES T. GRAHAM,  
C. SEDGWICK.